

## UNITED STATES PATENT OFFICE

2,261,851

## IRON ALLOY FOR CUTTING TOOLS

Leo Klüger, Vienna, Germany, assignor to Ferror  
Steel Corporation, of Luxembourg

No Drawing. Application October 31, 1938, Serial No. 238,026. In Germany November 3, 1937

## 1 Claim. (Cl. 75—126)

It has previously been proposed to make cutting tools, drills, reamers, milling and other tools, which must be made of specially hard material, from iron alloys which are capable of being cast and flow easily, the rough casting being substantially in the final shape required. These alloys have a somewhat high carbon content in order to ensure the fluidity necessary for casting; they also contain additions of tungsten, molybdenum and chromium. It has been found, however, that the behaviour of these steel alloys is such that they cannot be widely used in practice.

The cutting speed of these steels can not be increased up to that of high speed steels because the surface of the object to be machined is then not smooth but becomes wavy to some extent and a subsequent grinding process is necessary. It has also been found that these alloys must be hardened at high temperatures and the parts of the tool which are subjected to the greatest stress, namely the cutting edges, will not withstand such high temperatures but fuse away. Finally, it has also been found that erosion of the cutting edge takes place at red heat during working, for example during milling.

All these disadvantages are obviated when tools made of alloys in accordance with the present invention are used. In the alloys according to the invention a definite relationship is maintained between chromium on the one hand and the sum of all the other selected alloy additions on the other hand. Particular attention is drawn to the fact that milling cutters and other tools which are made from these alloys can be cast to the finished dimensions, ground and operated at high cutting speeds, notwithstanding which the machined surface remains quite even and smooth and does not require to be subsequently smoothed or ground as usual.

An alloy in accordance with the invention may consist for example of 6% chromium, 1% tungsten, 1% molybdenum, 1% cobalt, 0.5% manganese, 0.5% vanadium, carbon in an amount up to 1.5%, and the remainder iron. In this alloy the weight of the tungsten, molybdenum, cobalt, manganese, vanadium, and carbon amounts to substantially 92% of the weight of the chromium when the alloy contains 1.5% carbon.

A feature which is essential if the alloys are to have the properties desired is that the sum

of all the metallic and metalloid constituents excluding chromium amounts to 60% or more of the chromium content of the alloy. The parts by weight of the constituents contained in the alloy can therefore be varied, for example, in accordance with the following table without departing from the condition stated above and without impairing the usefulness of the alloy for the purpose in question.

| Cr      | W <sub>o</sub> | Mo      | Co      | Mn      | V <sub>a</sub> |
|---------|----------------|---------|---------|---------|----------------|
| Percent | Percent        | Percent | Percent | Percent | Percent        |
| 6.0     | 1.8            | 0.6     | 1.2     |         |                |
| 8.0     | 2.4            | 0.8     | 1.6     |         |                |
| 10.0    | 4.0            | 0.5     | 3.0     | 0.5     | 0.5            |

In the above table the weight of the alloying elements, other than chromium, ranges from 60% to 85% of the weight of the chromium.

These alloys flow easily so that milling cutters, drills and the like can be cast in their final shape. The alloys do not contract and expand very greatly under heat treatment. They also become so hard when hardened at a temperature of about 900° C. that their ability to cut at high working speeds is ensured; also the cutting edges do not fuse away. A milling cutter made of an alloy in accordance with the invention produces a smooth and even surface on the work, so that only a single machining of the work need be undertaken and subsequent grinding is not necessary.

Obviously the individual alloy additions which have been mentioned can be replaced by other substances, regard being paid to the relationship between atomic weight and proportions by weight, without departing from the scope of the invention. Alloys in which the chromium content differs from that given in the examples also fall within the invention provided the relationship between the chromium content and the sum of the remaining metallic or metalloid additions is maintained.

## I claim:

A steel alloy, adapted to be cast, for cutting tools, containing Cr about 10%, W<sub>o</sub> about 4%, Mo about 0.5%, Co about 3%, Mn about 0.5%, V<sub>a</sub> about 0.5%, C in an amount up to 1.5%, and the remainder Fe.

LEO KLÜGER.